

Oct. 30, 1928.

**1,689,312**

**R. R. WILLIAMS**

## METHOD OF INSULATING CONDUCTORS

Filed April 2, 1924

Fig. 1



Fig. 2



Inventor:  
Robert R. Williams,  
by E. Adams, Atty

Patented Oct. 30, 1928.

1,689,312

# UNITED STATES PATENT OFFICE.

ROBERT R. WILLIAMS, OF ROSELLE, NEW JERSEY, ASSIGNOR TO WESTERN ELECTRIC COMPANY, INCORPORATED, OF NEW YORK, N. Y., A CORPORATION OF NEW YORK.

## METHOD OF INSULATING CONDUCTORS.

Application filed April 2, 1924. Serial No. 703,660.

This invention relates to electrical conductors and more particularly to the insulated electrical conductors of submarine cables.

It is an object of the invention to improve the insulation of such conductors both electrically and mechanically and to apply the insulating material to the conductor in such a manner as not to deleteriously affect the conductor itself and in the case of a loaded conductor, to apply the insulating material so that the loading material with which the conductor is wrapped will not be subject to injury.

The use of hard rubber or semi-hard rubber as the material for insulating submarine conductors offers important advantages because of its low conductance, low dielectric constant and the fact that it is more rigid than soft rubber and therefore its osmotic swelling by water absorption is very limited. However, if the rubber compound is vulcanized on the conductor it is very difficult to prevent deformation of the insulation during the long vulcanizing process necessary and, furthermore, the extent of the sulphur attack on the conductor is objectionable during the long period of heating. Moreover vulcanization of the rubber compound on the conductor cannot be accomplished so as to give a satisfactory result in the case of a continuously loaded conductor of the type recently developed. In this conductor, a recently discovered alloy is employed for the loading material, such an alloy having a permeability at low magnetizing forces far in excess of that obtained with the best iron wire heretofore employed for continuous loading. However, to obtain the best results with this new alloy when used in a submarine cable, it is necessary to protect it from mechanical strains induced by hydrostatic pressure exerted on it at sea bottom and to protect against such strains it has been found desirable to impregnate the loaded conductor with an insulating compound such as liquid bitumen that fills all the interstices between adjacent turns of the loading material and between the loading material and the conductor itself and also in the case of a stranded conductor between adjacent strands of the conductor. To this end, it is preferable to employ an impregnating material which is fluid at the temperature encountered in great depths of water. Complete disclosures of the new loading material and its application to submarine cable con-

ductors are found in patents to G. W. Elmen No. 1,586,884 and O. E. Buckley Nos. 1,586,874 and 1,586,875, all issued on June 1, 1926. It is not satisfactory to vulcanize the rubber compound on a core of this type in which a layer of liquid bitumen is provided under the insulating material since the liquid bitumen mixes with the rubber compound during vulcanization and hardens to such an extent as to render it useless in protecting the loading material from subsequent strains.

To provide an insulated conductor having the desired characteristics, the invention contemplates the use of an insulating compound which is first vulcanized then rendered plastic and extruded in a continuous sheath about the conductor by means of heat and pressure.

In the accompanying drawing, Fig. 1 is a sectional view of an extruding press by means of which the plastic mass of prevulcanized rubber is extruded about the conductor, and Fig. 2 is a view of a continuously loaded conductor made in accordance with the features of this invention.

In practicing this invention, sheets of vulcanized hard rubber are rendered plastic by working them in standard rubber mills, the rolls of which are heated, or in some other equivalent manner. The term "hard rubber" is here used to also include these compositions sometimes referred to as "semi-hard rubber" in which the sulphur component may be as low as 15 per cent. In order that the vulcanized sheets may be more easily rendered sufficiently plastic to permit the material being extruded, it is desirable to include in the rubber compound a thermoplastic material such as a bitumen, preferably of one of the harder varieties. While the composition of the insulating compound will obviously depend largely upon the temperatures and pressures employed, a compound, which may be extruded at a temperature of 150° C. or somewhat less and with extruding pressures of from 1000 to 2000 pounds per square inch consists of approximately 60% rubber, 20% sulphur and 20% bitumen vulcanized at temperatures corresponding to 90 to 100 pounds steam pressure until the free sulphur content is reduced to .5 per cent or less in a manner such as is now commonly employed in the hard rubber industry. In place of or in addition to adding a bitumen to render the vulcanized compound more thermoplastic, it is possible to use, in whole or in part, the material made in

accordance with the process described in a copending application of Archie R. Kemp, Serial No. 725,691, filed July 12, 1924, which has issued as Patent No. 1,638,535 on August

5 9, 1927.

After the vulcanized sheets have been thoroughly worked by the heated rolls of the mill, the plastic mass 3 is fed into the hopper 4 of the extruding press shown in 10 Fig. 1 of the drawing. This press is provided with a tubular central portion 5 into which the extruding material passes as it leaves the hopper, being forced along by means of a rotating worm 6 driven by gear 7. 15 The gear and worm are provided with a hollow central portion through which the conductor to be insulated is driven at a predetermined rate by means not shown. As the conductor emerges through the end of 20 the worm 6, it passes through the compressed plastic mass and the die 9 held in position by a retaining plate 10 maintains the desired outer diameter of the insulated conductor. In order to maintain the insulating 25 material in a plastic condition until after it is extruded, the press is provided with jackets 11, 11 through which live steam is passed from pipes 12, 12. A steam pressure is preferably maintained so as to insure 30 a suitable temperature of approximately 150° C.

In Fig. 2 there is shown the finished conductor comprising a central core 15 surrounded by conductor strands 16, 16 about 35 which is helically wrapped the loading material 17 over which is placed a coating of liquid bitumen 18. The conductor completed thus far is passed through the extruding press where it is provided with a sheath 19 40 of prevulcanized insulating compound.

What is claimed is:

1. The method of insulating a conductor which consists in forming thereabout a contiguous and continuous single layer of prevulcanized hard rubber.
- 45 2. The method of insulating a conductor which consists in extruding thereabout prevulcanized hard rubber by the application of heat and pressure.
- 60 3. The method of insulating a conductor which consists in vulcanizing the insulating

material, rendering the vulcanized material plastic and extruding said material about the conductor by the application of heat and pressure.

55

4. The method of insulating a conductor with vulcanized hard rubber which method consists in rendering the vulcanized rubber plastic and immediately extruding said vulcanized rubber about the conductor by suitable application of heat and pressure.

60

5. The method of insulating a conductor with a vulcanizable material containing approximately 20% bitumens which method consists in vulcanizing the insulating material, rendering it plastic by milling with heated rolls, and immediately extruding said material about the conductor.

65

6. The method of insulating a conductor which consists in vulcanizing sheets of a rubber compound including hard bitumen vulcanized at a temperature corresponding to approximately 95 pounds steam pressure, rendering said compound plastic by milling with heated rolls, and extruding said compound about the conductor by means of the application of suitable heat and pressure.

70

7. The method of producing a conductor continuously loaded with magnetic material of high permeability and sensitive to mechanical strain which comprises applying the loading material to the conductor, impregnating the loaded conductor with a substance poorly adapted to remain in situ unchanged by the heat necessary for vulcanization, and forming thereabout a contiguous and continuous single layer of prevulcanized hard rubber.

75

8. The method of producing a layer of vulcanized insulating material upon a conductor loaded with strain sensitive magnetic material without detrimentally affecting the properties of a compound in which the loading material is imbedded to relieve it from strain which comprises first vulcanizing the insulating material, rendering it plastic, and then extruding it about the compound by the application of heat and pressure.

80

In witness whereof, I hereunto subscribe my name this 27th day of March A. D., 1924.

85

ROBERT R. WILLIAMS.

90

95